

## 1

3,830,723

### PROCESS FOR PREPARING HVI LUBRICATING OIL BY HYDROCRACKING A WAX

Peter Ladeur and Gerrit Van Gooswilligen, Amsterdam, Netherlands, assignors to Shell Oil Company, New York, N.Y.

No Drawing. Filed Mar. 21, 1973, Ser. No. 343,614  
Claims priority, application Netherlands, Apr. 6, 1972,  
7204581; Dec. 19, 1972, 7217257

Int. Cl. C10g 13/06

U.S. CL. 208—108

11 Claims

#### ABSTRACT OF THE DISCLOSURE

A lubricating oil meeting the SAE-10W/30 specification is prepared from wax obtained from a de-asphalting residual mineral oil fraction by hydrocracking at 325–425° C. over a fluorine-containing alumina-supported mixed sulfide catalyst to give a liquid product containing 25–85% wt. material boiling above 400° C., isolating a residual fraction having an initial boiling point between 350 and 470° C., and dewaxing that fraction.

#### Background of the Invention

The invention relates to a process for the preparation of a lubricating oil having a dynamic viscosity at –17.8° C. of at most 24 P (Poise) and a kinematic viscosity at 98.9° C. of at least 7.0 cst. (centistokes), by hydrocracking of wax.

According to the SAE classification, lubricating oils for combustion engines are divided on the basis of their viscosity into two groups which are designated by the names winter grade and normal grade. Each of these groups is subdivided into a number of classes. Lubricating oils which are classed as winter grade are designated by the letter W, preceded by a numeral, for example an SAE-5W, –10W or –20W oil. These oils have to satisfy a certain requirement as regards their dynamic viscosity at –17.8° C. Lubricating oils classed as normal grade are designated merely by a numeral, for example an SAE-20, –30, –40 or –50 oil. These oils must satisfy a certain requirement as regards their kinematic viscosity at 98.9° C. Lubricating oils which only belong to one SAE class (either of the winter grade or of the normal grade) are designated as single grade lubricating oils. Examples of widely used single grade lubricating oils are SAE-20 and SAE-30 oils.

In addition to the single grade lubricating oils, lubricating oils are also known which satisfy the viscosity requirement both of a class of the winter grade and the viscosity requirement of a class of the normal grade. When used as motor oil these multigrade lubricating oils have the advantage that in winter they are sufficiently thin to cause no difficulties when starting the engine from cold, and sufficiently thick at the temperature of the running engine to lubricate properly. An important class of the multigrade lubricating oils is that of the 10W/30 oils, which satisfy both the viscosity requirement for the SAE-10W class

## 2

(dynamic viscosity at –17.8° C. at least 12 P and at most 24 P, measured according to ASTM Standard D2602/71) and the viscosity requirement for the SAE-30 class (kinematic viscosity at 98.9° C. at least 9.6 cst. and at most 12.9 cst., measured according to ASTM Standard D 445/71).

The preparation of multigrade lubricating oils in the 10W/30 class is effected in practice by incorporating a number of additives with quality-improving properties in a base oil consisting of a lubricating oil or a blend of lubricating oils having a high viscosity index obtained in the conventional manner or by hydrocracking, which base oil in itself does not satisfy the 10W/30 specification.

The preparation of high-viscosity index lubricating oils in the conventional manner is carried out as follows. A paraffinic petroleum crude oil is separated by distillation at atmospheric pressure into a number of distillate fractions (in particular successively into one or more gasoline, kerosine and light gasoil fractions) and a residue (known as long residue). This long residue is then separated by distillation at reduced pressure into a number of distillate fractions (in particular successively into one or more heavy gasoil, spindle oil, light machine oil and medium heavy machine oil fractions) and a residue (known as short residue). From the lubricating oil fractions obtained during the distillation at reduced pressure, the corresponding lubricating oils are prepared by refining. The refining of the spindle oil fraction, light machine oil fraction and medium heavy machine oil fraction is effected by removing aromatics and wax from these fractions. In refining the short residue, asphalt is first of all removed from the residue. From the deasphalting oil thus obtained, aromatics and wax are subsequently removed. The residual lubricating oil prepared in this way is designated as bright stock. The wax obtained during refining of the various lubricating oil fractions is designated as distillate or residual slack wax, depending on the type of lubricating oil fraction from which are derived.

The preparation of high viscosity-index lubricating oils by hydrocracking is carried out as follows. A heavy fraction of a paraffinic petroleum crude oil such as a heavy distillate or a deasphalting oil is passed over a suitable catalyst under hydrocracking conditions. One or more lubricating oil fractions are separated by distillation from the hydrocracked product. From the lubricating oil fractions obtained in this way the corresponding lubricating oils are prepared by removing wax from these fractions.

The lubricating oils prepared in the manner described above, may, either as such or after blending, serve as base oils for the preparation of 10W/30 oils. As stated previously, the 10W/30 oils are prepared by incorporating in the base oils a number of additives with quality-improving properties. These additives may be divided into two groups. The first group comprises inter alia the additives to inhibit oxidation (anti-oxidants), corrosion (corrosion inhibitors), the formation of foam (anti-foaming agents) and deposits in the engine (detergents), as well as additives to improve the lubricating effect at high pressure (extreme pressure additives). The additives belonging to this group generally have a molecular weight which does

not exceed a value of 10,000 and is generally far below this value. The lubricating oil additive packages marketed by a number of manufacturers are generally composed of additives of this type.

The incorporation of such a lubricating oil additive package in a base oil has only a slight effect on the viscosity index of this oil, even if the additive package is used in a rather high concentration. Depending on the composition of the additive package which is incorporated in the oil, the viscosity index of the oil either remains constant, increases somewhat, or may even decrease slightly. Whenever reference is made hereinafter to "additive package" this reference should be taken as meaning a blend of lubricating oil additives belonging to the above-mentioned first group, which blend has the property that when it is incorporated in a base oil in a concentration of 15% by weight, the viscosity index of this formulation (85% by weight of base oil + 15% by weight of blend) is not more than 5 units higher than the viscosity index of the base oil.

The second group of additives having quality-improving properties used in the preparation of 10W/30 oils includes the viscosity index improvers. The additives in this group generally have a molecular weight exceeding a value of 10,000 and frequently far in excess of this value.

There are serious drawbacks to the use of viscosity index improvers for the preparation of the present multi-grade lubricating oils. In the first place, the high molecular weight compounds (generally polyalkylacrylates and polyalkylmethacrylates) used for this purpose are insufficiently resistant to the shearing forces which occur in the engine and moreover they are sensitive to oxidation. As a result of this the polymers are decomposed in the engine and, in addition to fouling of the engine by decomposition products, a permanent decrease in the viscosity of the oil takes place. Furthermore, a temporary loss of viscosity occurs while the lubricating oil is being used because the polymers become oriented under the influence of the shearing forces in the engine, which leads to reduced internal friction. As the shearing forces increase the apparent viscosity of the polymer-containing oil approaches that of the polymer-free oil.

It is clear from the above that there is an urgent need for lubricating oils which satisfy the 10W/30 specification without the addition of a polymeric viscosity index improver. Attempts to prepare such oils in the conventional manner, i.e. by distillation and refining, have remained without success.

#### THE INVENTION

It has now been found that lubricating oils which satisfy the 10W/30 specification either as such or after the addition of an additive package but without the addition of a polymeric viscosity index improver, can be prepared in a yield of more than 15% wt., based on the feed, by catalytic hydrocracking of wax, provided that the following requirements regarding starting material, catalyst, hydrocracking conditions and product separation are met.

The starting material consists of wax of which more than 30% wt. boils above 520° C. and which is obtained during the dewaxing of a residual mineral oil fraction.

The hydrocracking catalyst contains nickel sulfide and/or cobalt sulfide and in addition molybdenum sulfide and/or tungsten sulfide supported on alumina, and the catalyst also contains fluorine.

The hydrocracking process is carried out at a temperature between 325° C. and 425° C. and further under such conditions that the resultant liquid reaction product consists of 25% to 95% by weight of components having a boiling point in excess of 400° C.

The reaction product is separated by distillation into one or more light fractions and a residual fraction having an initial boiling point between 350° C. and 470° C. and the desired lubricating oil is prepared from the residual fraction by means of dewaxing.

The lubricating oils prepared in this manner which satisfy the 10W/30 specification either as such or after the addition of an additive package, but without the addition of a polymeric viscosity index improver, may be characterized as lubricating oils having a dynamic viscosity of at most 24 P at -17.8° C. (measured according to ASTM standard D 2602/71) and a kinematic viscosity of at least 7.0 and preferably of at least 8.4 cst. at 98.9° C. (measured according to ASTM standard D 445/71).

The wax used as starting material in the process according to the invention is preferably obtained as by-product during the preparation of lubricating oil in a conventional manner. As was explained above, in the preparation of lubricating oil in a conventional manner a residual lubricating oil is prepared by refining. This refining comprises the removal of asphalt, aromatics and wax. This wax is the preferred starting material in the process according to the invention. Before the residual lubricating oil fraction can be dewaxed, asphalt first has to be removed therefrom. De-asphalting can be carried out by treating the residual lubricating oil fraction with a low boiling paraffinic hydrocarbon, such as ethane, propane, butane or pentane, propane being preferred. Aromatics and wax are subsequently removed from the deasphalting oil obtained in this way. The removal of aromatics from the deasphalting oil may be carried out by treating the deasphalting oil with a selective solvent for aromatic hydrocarbons such as furfural, phenol, cresol, or Chlorex, furfural being preferred. Finally wax is removed from the resultant oil, which is known as bright stock waxy raffinate. Dewaxing of the oil may be carried out by cooling the oil in the presence of a solvent. Dewaxing is preferably carried out with a mixture of methyl ethyl ketone and toluene at a temperature between -10° C. and -40° C. and a solvent-to-oil volume ratio between 1:1 and 10:1. The sequence in which the removal of aromatics and wax from the deasphalting oil takes place is in principle arbitrary, but in order to minimize the volume of oil which is cooled during dewaxing, the dewaxing should preferably only be carried out after the aromatics have been removed from the deasphalting oil.

Preferably the wax used as a starting material will contain less than 35% by weight of oil. It is also preferred that the wax which is hydrocracked has been obtained from a de-asphalting lubricating oil fraction which after dewaxing at -30° C. has a viscosity index of at least 55 and in particular of at least 70.

The hydrocracking catalysts which are used in the process according to the invention are fluorine-containing sulfidic catalysts containing nickel and/or cobalt and in addition molybdenum and/or tungsten on alumina as carrier. Preferred catalyst are those which contain 0.025-0.8 gram atoms and in particular 0.05-0.7 gram atoms of nickel and/or cobalt and 0.05-0.5 gram atoms and in particular 0.1-0.4 gram atoms of molybdenum and/or tungsten per 100 grams of alumina. The atomic ratio between nickel and/or cobalt on the one hand and molybdenum and/or tungsten on the other is preferably between 0.1:1 and 2:1, and in particular between 0.2:1 and 1.6:1.

The metals may be incorporated into the present catalysts by any method known in the art for the preparation of catalysts containing several components on a carrier, for example by co-impregnation of alumina in one or more stages with an aqueous solution containing salts of the metals concerned. The catalysts are used in sulfidic form. The catalysts may be sulfided by any method known in the art for the sulfiding of catalysts, for example by contacting the catalysts with a mixture of hydrogen and hydrogen sulfide or with hydrogen and a sulfur-containing hydrocarbon oil, such as a sulfur-containing gas oil.

In addition to the metals nickel and/or cobalt and molybdenum and/or tungsten, the catalyst used in the process according to the invention should also contain fluorine.

The incorporation of fluorine into the catalysts may in principle be carried out in two manners. Fluorine may be incorporated into the catalyst by impregnating the latter during or after the preparation with a suitable fluorine compound such as ammonium fluoride. It is also possible to incorporate fluorine into the catalyst by in situ fluorination of the catalyst in an early stage of the hydrocracking process for which the catalyst is used (for example during or after the start-up of the process). In situ fluorination of the catalysts may be carried out by adding a suitable fluorine compound, such as o-fluoro toluene or difluoro ethane, to the gas and/or liquid stream which is passed over the catalyst. In a number of cases it may be preferred to incorporate at least some of the fluorine in the catalyst by in situ fluorination. The quantity of fluorine contained in the present catalyst is preferably 0.5 to 7% by weight. In addition to nickel and/or cobalt, molybdenum and/or tungsten and fluorine, the catalysts used in the process according to the invention may further contain promoters such as boron and phosphorus.

In the preparation of lubricating oil by hydrocracking of wax according to the invention, very favorable results are achieved by using one of the following catalysts.

(a) A catalyst prepared by impregnating alumina with a solution containing one or more nickel and/or cobalt compounds, one or more molybdenum and/or tungsten compounds, phosphate ions and peroxide ions, followed by drying and calcination of the composition.

(b) A catalyst prepared by incorporating into an alumina hydrogel one or more nickel and/or cobalt compounds and one or more molybdenum and/or tungsten compounds in a sufficient concentration to impart to the finished catalyst a metal content, expressed as metal oxides of 30% to 65% by weight, followed by drying and calcination of the composition; the alumina hydrogel into which the metal compounds are incorporated should, after drying and calcination, yield a xerogel, i.e., the calcined hydrogel before metal compounds are added, with a compacted bulk density of 0.75 to 1.6 g./ml. and a pore volume of 0.15 to 0.5 ml./g.

(c) A catalyst prepared by treating a composition containing alumina, water, one or more water-soluble salts of nickel and/or cobalt with one or more water-soluble salts of molybdenum and/or tungsten, with a hydrogen sulfide-containing gas at a temperature below 150° C. and subsequently heating the material in a hydrogen-containing gas to a final temperature in excess of 200° C.; the quantity of water present in the composition which is treated with the hydrogen sulfide-containing gas should correspond with the quantity of water present in the composition after drying in a dry gas at 110° C., increased by 20% to 120% of the quantity of water which the dried composition can absorb in the pores of the carrier at 20° C.

The catalysts which are used in the hydrocracking process according to the invention preferably contain as catalytically active metal components nickel and molybdenum or nickel and tungsten.

The hydrocracking process should be carried out at a temperature between 325° C. and 425° C. and in addition under such conditions that 25% to 95% by weight of the resultant liquid reaction product consists of components having a boiling point in excess of 400° C. Suitable hydrocracking conditions are a pressure of 10 to 250 bar, a space velocity of 0.2 to 5 kg. of feed per litre of catalyst per hour and a hydrogen/feed ratio of 100 to 5000 Nl. of hydrogen per kg. of feed. The hydrocracking process is preferably carried out under the following conditions: a temperature of 360° C. to 415° C., a pressure of 25 to 200 bar, a space velocity of 0.5 to 1.5 kg. of feed per litre of catalyst per hour and a hydrogen/feed ratio of 500 to 2500 Nl. per kg. of feed.

The wax is converted by hydrocracking into a liquid product, 25% to 95% wt. of which consists of components

having a boiling point over 400° C. and the reaction product is separated by distillation into one or more light fractions and a residual fraction having an initial boiling point between 350° C. and 470° C. Preferably, the wax 5 is converted by hydrocracking into a liquid product, 40% to 70% by weight of which consists of components having a boiling point in excess of 400° C. and a residual fraction having an initial boiling point between 390° C. and 450° C. is separated by distillation from the reaction 10 product.

To prepare a suitable lubricating oil the residual fraction must be dewaxed. Dewaxing is preferably carried out by cooling the oil in presence of a solvent. Very suitable for this purpose is a mixture of methyl ethyl ketone 15 and toluene at a temperature between -10° C. and -40° C. and a solvent-to-oil volume ratio between 1:1 and 10:1. In order to increase the yield of desired lubricating oil, it is preferred to recycle to the hydrocracking reactor at least a portion of the wax separated during dewaxing of the residual fraction of the hydrocracked 20 product.

The process according to the invention enables lubricating oils to be prepared which as such, i.e., without additive having been incorporated therein, meet the 10W/30 25 specification. The process according to the invention moreover enables lubricating oils to be prepared which as such do not meet the 10W/30 specification, but from which in a simple manner, without the use of high molecular viscosity index improvers, a 10W/30 oil can be prepared by incorporating therein a certain quantity of an additive package. The commercial additive packages which 30 are at present used in practice in the preparation of multi-grade lubricating oils comprise a number of compounds each of which individually have the property that when 35 they are incorporated in a lubricating oil they improve the quality of this lubricating oil in one or more respects. Examples of additives which are found in these additive packages are inter alia anti-oxidants, rust inhibitors, corrosion inhibitors, anti-wear agents, anti-foam agents, detergents, metal passivators and extreme pressure additives. 40 In some cases, several quality-improving properties are combined in a single additive. If the lubricating oils prepared according to the invention are intended for use as motor oils, it is advisable to incorporate therein a certain quantity of additive package, even if the lubricating oil as such already meets the 10W/30 specification. In the preparation of 10W/30 oils according to the invention, it is preferred to incorporate such a quantity of 45 the additive package in the base oil (which may or may not meet the 10W/30 specification) that an oil composition 50 is obtained which comprises 87.5% to 95% by weight of base oil and 5% to 12.5% of additives.

The invention will now be elucidated with reference to the following Examples.

#### Example I

Eight catalysts (A-H) were used in hydrocracking experiments to prepare lubricating oil from six residual waxes (I-VI). The catalyst and feeds are described in 55 more detail below.

Catalyst A: Ni/Mo/F/Al<sub>2</sub>O<sub>3</sub> catalyst with a pore volume of 0.44 ml./g. and a specific surface area of 117.1 m<sup>2</sup>/g. containing 6 parts by weight of nickel, 30 parts by weight of molybdenum and 7.5 parts by weight 60 of fluorine per 100 parts by weight of alumina. This catalyst had been prepared by co-impregnation of alumina with an aqueous solution of ammonium molybdate, nickel nitrate and ammonium fluoride. After the degree of wetting had been set at 100%, the composition was first treated for 16 hours with H<sub>2</sub>S at 15 bar and 75° C., subsequently heated in 2 hours to 400° C. in a stream of H<sub>2</sub>S-containing H<sub>2</sub> (9% v. H<sub>2</sub>S, 10 bar, 25,000 Nl. 1<sup>-1</sup>, hour<sup>-1</sup>) and finally kept for approximately 2 hours in this gas stream. The expression "degree of wetting" used 65 above relates to the quantity of water present in the com-

position in addition to the quantity of water which is present therein after drying of the composition in a drying gas at 110° C. The degree of wetting is expressed as a percentage of the quantity of water which the dried composition can absorb in the pores of the carrier at 20° C.

Catalyst B: Ni/Mo/F/Al<sub>2</sub>O<sub>3</sub> catalyst with a pore volume of 0.23 ml./g. and a specific surface area of 63.0 m.<sup>2</sup>/g. containing 6 parts by weight of nickel, 30 parts by weight of molybdenum and 7.5 parts by weight of fluorine per 100 parts by weight of alumina. This catalyst was prepared in the same way as catalyst A except that another type of alumina was used.

Catalyst C: Ni/W/F/Al<sub>2</sub>O<sub>3</sub> containing 5 parts by weight of nickel, 38 parts by weight of tungsten per 100 parts by weight of alumina and 2.4% by weight of fluorine. This catalyst was prepared in the same manner as catalysts A and B, except that a fluorine-free impregnation liquid was used which contained ammonium-tungstate and nickel nitrate and that fluorine was incorporated into the catalyst by fluorination in situ.

Catalyst D: Ni/Mo/P/Al<sub>2</sub>O<sub>3</sub> catalyst containing 4.2 parts by weight of nickel, 17.7 parts by weight of molybdenum and 3.1 parts by weight of phosphorous per 100 parts by weight of alumina and 1.6% by weight of fluorine. This catalyst was prepared by co-impregnation of alumina with an aqueous solution containing nickel nitrate, phosphoric acid, ammonium molybdate and hydrogen peroxide, followed by drying and calcination of the composition. Fluorine was incorporated into the catalyst by fluorination in situ.

Catalyst E: Ni/W/F/Al<sub>2</sub>O<sub>3</sub> catalyst containing 31 parts by weight of nickel, 58 parts by weight of tungsten and 7.5 parts by weight of fluorine per 100 parts by weight of alumina.

Catalyst F: Ni/W/F/Al<sub>2</sub>O<sub>3</sub> catalyst containing 31 parts by weight of nickel and 58 parts by weight of tungsten per 100 parts by weight of alumina and 6% by weight of fluorine.

Catalyst G: Ni/W/F/Al<sub>2</sub>O<sub>3</sub> catalyst containing 37 parts by weight of nickel and 70 parts by weight of tungsten per 100 parts by weight of alumina and 4.3% by weight of fluorine.

The catalysts E, F and G were prepared by mixing an alumina hydrogel with an aqueous solution containing nickel nitrate, ammonium tungstate and ammonium fluoride, the pH of which solution had been brought to 6.5 with the aid of 25% of ammonia. The mixture was heated to 80° C.; the gel was filtered, extruded, dried and calcined. After drying and calcining, the alumina hydrogel used in the preparation of these catalysts yielded a xerogel with a compacted bulk density between 0.75 and 1.6 g./ml. and a pore volume between 0.15 and 0.5 ml./g.

Catalyst H: Ni/W/F/Al<sub>2</sub>O<sub>3</sub> catalyst containing 10 parts by weight of nickel and 60 parts by weight of tungsten per 100 parts by weight of alumina and 4.5% by weight of fluorine. This catalyst was prepared by co-impregnation of alumina with an aqueous solution containing nickel nitrate and ammonium tungstate and subsequent drying and calcination. Fluorine was incorporated into the catalyst by fluorination in-situ.

In situ fluorination of the catalysts C, D and H was carried out by adding o-fluorotoluene to the feed during the initial stage of the hydrocracking process.

Feed I (Bright stock slack wax): Wax obtained in dewaxing a residual lubricating oil fraction (1) which had previously been deasphalting with propane and extracted with furfural. Initial boiling point of the wax: 520° C. Oil content of the wax: 19.7% by weight. VI of the oil obtained after the wax had been deoiled: 97. Sulfur content of the wax: 0.34% by weight.

Feed II (DOA slack wax): Wax obtained in dewaxing a residual lubricating oil fraction (1) which had pre-

viously been deasphalting with propane. Initial boiling point of the wax: 520° C. Oil content of the wax: 9.8% by weight. VI of the oil obtained after deoiling the wax: 78. Sulfur content of the wax: 0.85% by weight.

Feed III (Bright stock slack wax): Wax obtained in dewaxing a residual lubricating oil fraction (1) which had previously been deasphalting with propane and extracted with furfural. Initial boiling point of the wax: 520° C. Oil content of the wax: 21.1% by weight. VI of the oil obtained after the wax had been deoiled: 98. Sulfur content of the wax: 0.66% by weight.

Feed IV (Wax from hydrocracked bright stock slack wax): Wax obtained in dewaxing a residual fraction of a hydrocrackate which had been prepared by hydrocracking of wax obtained in dewaxing a residual lubricating oil fraction (1) which had previously been deasphalting with propane and extracted with furfural. Initial boiling point of the feed wax: 390° C. Of this wax 92.5% by weight boiled above 520° C. Oil content of the feed wax: 6% by weight. VI of the oil obtained after the feed wax had been deoiled: 149. Sulfur content of the feed wax: 20 p.p.m.w.

Feed V (Wax from hydrocracked bright stock slack wax): Wax obtained in dewaxing a residual fraction of a hydrocrackate which had been prepared by hydrocracking of wax obtained in dewaxing a residual lubricating oil fraction (1) which had previously been deasphalting with propane and extracted with furfural. Initial boiling point of the feed: 520° C. Oil content of the feed wax: 7% by weight. VI of the oil obtained after the feed wax had been deoiled: 150. Sulfur content of the feed wax: 20 p.p.m.w.

Feed VI (Wax from mildly hydrocracked DAO): Wax obtained in dewaxing a residual fraction of a hydrocrackate which had been prepared by mildly hydrocracking (25% by weight of the hydrocrackate boiled below the initial boiling point of the feed) of a residual lubricating oil fraction (1) which had previously been deasphalting with propane. Initial boiling point of the feed wax: 520° C. Oil content of the feed wax: 21% by weight. VI of the oil obtained after the feed was deoiled: 95. Sulfur content of the feed wax: 500 p.p.m.w.

The six residual lubricating oil fractions from which the feeds I-VI were prepared had been obtained as residue during distillation various paraffinic crude oils. Dewaxing was carried out by cooling the oil to a temperature of -30° C. in the presence of a 1:1 mixture of methyl ethyl ketone and toluene.

The viscosity indices mentioned in this patent application were determined by ASTM standard D 2270.

## Example 2

The hydrocracking experiments 1-26 were carried out under the following conditions:

pressure: 150 bar, except for experiment 7; this experiment was carried out at a pressure of 50 bar,  
temperature: 375-410° C.,  
space velocity: 11.1<sup>-1</sup>.hour<sup>-1</sup>,  
hydrogen/feed ratio: 2000 Nl.1<sup>-1</sup>,  
catalyst bed: 100 ml.

The catalysts were used in the sulfidic form. Sulfiding of the catalysts D-G was carried out by contacting them with hydrogen and a sulfur-containing gas oil. From the hydrocracked products, residual fractions having an initial boiling point between 365° C. and 440° C. were separated by distillation. From the residual fractions the corresponding lubricating oils were prepared by dewaxing the fractions. Dewaxing was carried out by cooling the oil to a temperature of -30° C. in the presence of a 1:1 mixture of methyl ethyl ketone and toluene.

The results of the hydrocracking experiments 1-26 are shown in Table A.

TABLE A

| Exp. No. | Cat. No. | Feed No. | Hydro-cracking temp., °C. | Quantity of material boiling above 400° C. present in the liquid reaction products percent wt. | Initial boiling point of the separated residual lub. oil fraction, °C. | Properties of the dewaxed residual lubricating oil fraction |     |                                          |
|----------|----------|----------|---------------------------|------------------------------------------------------------------------------------------------|------------------------------------------------------------------------|-------------------------------------------------------------|-----|------------------------------------------|
|          |          |          |                           |                                                                                                |                                                                        | Yield based on feed, percent wt.                            | VI  | Kinematic viscosity at 98.9° C., est. P. |
| 1        | G        | III      | 390                       | 70                                                                                             | 400                                                                    | 43                                                          | 144 | 9.8                                      |
| 2        | F        | III      | 390                       | 67                                                                                             | 400                                                                    | 33                                                          | 142 | 9.9                                      |
| 3        | D        | I        | 394                       | 67                                                                                             | 400                                                                    | 27                                                          | 142 | 9.7                                      |
| 4        | B        | I        | 405                       | 72                                                                                             | 400                                                                    | 35                                                          | 146 | 9.7                                      |
| 5        | A        | I        | 402                       | 71                                                                                             | 400                                                                    | 36                                                          | 143 | 9.7                                      |
| 6        | C        | II       | 398                       | 70                                                                                             | 400                                                                    | 27                                                          | 154 | 9.7                                      |
| 7        | E        | II       | 394                       | 69                                                                                             | 400                                                                    | 28                                                          | 143 | 9.7                                      |
| 8        | B        | I        | 405                       | 72                                                                                             | 400                                                                    | 35                                                          | 146 | 9.8                                      |
| 9        | D        | III      | 397                       | 67                                                                                             | 420                                                                    | 26                                                          | 144 | 9.7                                      |
| 10       | G        | IV       | 375                       | 86                                                                                             | 390                                                                    | 30                                                          | 154 | 10.0                                     |
| 11       | G        | V        | 375                       | 88                                                                                             | 390                                                                    | 28                                                          | 155 | 9.9                                      |
| 12       | A        | I        | 410                       | 60                                                                                             | 400                                                                    | 37                                                          | 143 | 8.7                                      |
| 13       | A        | I        | 395                       | 77                                                                                             | 365                                                                    | 37                                                          | 143 | 9.3                                      |
| 14       | A        | I        | 400                       | 72                                                                                             | 385                                                                    | 38                                                          | 142 | 9.4                                      |
| 15       | A        | I        | 405                       | 65                                                                                             | 410                                                                    | 37                                                          | 145 | 9.4                                      |
| 16       | A        | I        | 410                       | 44                                                                                             | 440                                                                    | 26                                                          | 144 | 9.4                                      |
| 17       | B        | I        | 405                       | 72                                                                                             | 390                                                                    | 36                                                          | 146 | 9.4                                      |
| 18       | D        | III      | 397                       | 67                                                                                             | 400                                                                    | 27                                                          | 145 | 8.9                                      |
| 19       | D        | III      | 397                       | 67                                                                                             | 405                                                                    | 27                                                          | 145 | 9.1                                      |
| 20       | D        | III      | 397                       | 67                                                                                             | 410                                                                    | 27                                                          | 145 | 9.3                                      |
| 21       | G        | IV       | 380                       | 83                                                                                             | 390                                                                    | 41                                                          | 154 | 8.9                                      |
| 22       | G        | V        | 380                       | 83                                                                                             | 390                                                                    | 41                                                          | 156 | 9.2                                      |
| 23       | H        | VI       | 385                       | 56                                                                                             | 400                                                                    | 40                                                          | 149 | 8.5                                      |
| 24       | G        | III      | 400                       | 46                                                                                             | 400                                                                    | 31                                                          | 148 | 8.6                                      |
| 25       | F        | I        | 390                       | 63                                                                                             | 400                                                                    | 38                                                          | 146 | 8.6                                      |
| 26       | A        | II       | 410                       | 72                                                                                             | 400                                                                    | 35                                                          | 149 | 8.4                                      |

The experiments 1-26 shown in the Table A are all hydrocracking experiments according to the invention. Each of these experiments yields more than 15% wt., based on the feed, of a lubricating oil having a dynamic viscosity of at most 24 P at -17.8° C. and a kinematic viscosity of at least 7.0 cst. at 98.9° C. The lubricating oils prepared according to the experiments 1-11 meet the 10W/30 specification (dynamic viscosity at -17.8° C. at

35

Incorporation of additive package A in the lubricating oil yields a lubricating oil composition containing 92.5% wt. of the base oil and 7.5% wt. of the additive package. Incorporation of additive package B in the lubricating oil yields a lubricating oil composition containing 89.9% wt. of the base oil and 10.1% wt. of the additive package. The properties of the prepared oil compositions are shown in Table B.

TABLE B

| Base oil prepared according to exp. No. | Properties of the base oil without additive package |                                          |                                    | Properties of a composition comprising 92.5% wt. of the base oil and 7.5% wt. of the additive package A |                                          |                                    | Properties of a composition comprising 89.9% wt. of the base oil and 10.1% wt. of the additive package B |                                          |                                    |
|-----------------------------------------|-----------------------------------------------------|------------------------------------------|------------------------------------|---------------------------------------------------------------------------------------------------------|------------------------------------------|------------------------------------|----------------------------------------------------------------------------------------------------------|------------------------------------------|------------------------------------|
|                                         | VI                                                  | Kinematic viscosity at 98.9° C., est. P. | Dynamic viscosity at -17.8° C., P. | VI                                                                                                      | Kinematic viscosity at 98.9° C., est. P. | Dynamic viscosity at -17.8° C., P. | VI                                                                                                       | Kinematic viscosity at 98.9° C., est. P. | Dynamic viscosity at -17.8° C., P. |
| 12                                      | 143                                                 | 8.7                                      | 18                                 | 140                                                                                                     | 9.9                                      | 24                                 | 143                                                                                                      | 9.8                                      | 22                                 |
| 13                                      | 143                                                 | 9.3                                      | 22                                 | 139                                                                                                     | 10.0                                     | 23                                 | 145                                                                                                      | 9.9                                      | 21                                 |
| 14                                      | 142                                                 | 9.4                                      | 21                                 | 142                                                                                                     | 10.0                                     | 22                                 | 145                                                                                                      | 10.1                                     | 22                                 |
| 15                                      | 145                                                 | 9.4                                      | 20                                 | 142                                                                                                     | 10.0                                     | 21.5                               | 145                                                                                                      | 10.4                                     | 23                                 |
| 16                                      | 144                                                 | 9.4                                      | 21                                 | 141                                                                                                     | 10.0                                     | 156                                | 154                                                                                                      | 10.3                                     | 19                                 |
| 17                                      | 146                                                 | 9.4                                      | 19                                 | 143                                                                                                     | 10.0                                     | 21                                 | 147                                                                                                      | 10.3                                     | 23                                 |
| 18                                      | 145                                                 | 8.9                                      | 17.5                               | 143                                                                                                     | 9.7                                      | 21                                 | 145                                                                                                      | 9.9                                      | 21                                 |
| 19                                      | 145                                                 | 9.1                                      | 18                                 | 143                                                                                                     | 9.7                                      | 21                                 | 145                                                                                                      | 10.1                                     | 22                                 |
| 20                                      | 145                                                 | 9.3                                      | 19                                 | 143                                                                                                     | 9.9                                      | 21.5                               | 145                                                                                                      | 10.4                                     | 23                                 |
| 21                                      | 154                                                 | 8.9                                      | 14                                 | 155                                                                                                     | 9.8                                      | 17.5                               | 156                                                                                                      | 9.9                                      | 18                                 |
| 22                                      | 156                                                 | 9.2                                      | 15                                 | 155                                                                                                     | 9.8                                      | 17.5                               | 154                                                                                                      | 10.3                                     | 19                                 |
| 23                                      | 149                                                 | 8.5                                      | 16                                 | 144                                                                                                     | 10.4                                     | 22.5                               | 149                                                                                                      | 9.6                                      | 20                                 |
| 8                                       | 146                                                 | 9.8                                      | 20                                 | 144                                                                                                     | 10.4                                     | 22.5                               | 147                                                                                                      | 10.9                                     | 24                                 |
| 9                                       | 144                                                 | 9.7                                      | 21                                 | 142                                                                                                     | 10.4                                     | 23.5                               | 157                                                                                                      | 11.1                                     | 22                                 |
| 10                                      | 154                                                 | 10.0                                     | 18                                 | 156                                                                                                     | 10.6                                     | 20.5                               | 154                                                                                                      | 11.0                                     | 2                                  |
| 11                                      | 155                                                 | 9.9                                      | 18                                 | 155                                                                                                     | 10.6                                     | 21                                 | 154                                                                                                      | 11.0                                     |                                    |

least 12 P and at most 24 P and kinematic viscosity at 98.9° C. at least 9.6 cst. and at most 12.9 cst.) as such, i.e., without the incorporation of additives.

60

## Example 3

An additive package was incorporated in the lubricating oils prepared according to the experiments 12-23 which do not meet the 10W/30 specification and in the lubricating oils prepared according to the experiments 8 and 11 which do meet the 10W/30 specification. Two additive packages were used, designated as additive package A and additive package B. These additive packages differ as regards the chemical composition of the additives which they contain but both have substantially the same effect, namely: anti-oxidation, rust-inhibition, wear resistance, corrosion inhibition, foam inhibition, metal passivation, improvement of the lubricating effect as high pressure and inhibition of deposits in the engine.

The results given in Table B show that lubricating oils prepared according to the invention which as such do not meet the 10W/30 specification (compare exp. 12-23) may be formulated to 10W/30 oils in a simple manner, without the addition of the customary high-molecular weight viscosity improvers, by the incorporation of the additive package A or B. Incorporation of these additive packages in a lubricating oil prepared according to the invention which already meets the 10W/30 specification (compare exp. 8-11) yields a 10W/30 oil of better quality.

## Example 4

In the process according to the invention it is essential that a fluorine-containing sulfidic catalyst be used which contains nickel and/or cobalt and in addition molybdenum and/or tungsten on alumina as carrier. To demonstrate the importance of fluorine a Ni/Mo/P/Al<sub>2</sub>O<sub>3</sub> catalyst containing 4.2 parts by weight of nickel, 17.7 parts

11

by weight of molybdenum and 3.1 parts by weight of phosphorous per 100 parts by weight of alumina (catalyst D without fluorine) was used for hydrocracking feed I. The conditions were the same conditions as were used in experiment 3, that the hydrocracking temperature was 445° C. The lubricating oil was processed in the same manner as in experiment 3. Table C compares the results of experiment 27 with those of experiment 3.

TABLE C

| Experiment number | Hydro-cracking temp., °C. | Properties of the dewaxed residual lubricating oil fraction |     |                                       |                                    |
|-------------------|---------------------------|-------------------------------------------------------------|-----|---------------------------------------|------------------------------------|
|                   |                           | Yield based on feed, percent wt.                            | VI  | Kinematic viscosity at 98.9° C., cst. | Dynamic viscosity at -17.8° C., P. |
| 27-----           | 445                       | 12                                                          | 140 | 9.1                                   | 22                                 |
| 3-----            | 394                       | 27                                                          | 142 | 9.7                                   | 23                                 |

The results shown in Table C demonstrate the unsuitability of the fluorine-free catalyst for the present purpose. At a hydrocracking temperature of 394° C., the fluorine-containing catalyst gives a lubricating oil yield of 27% by weight; at a hydrocracking temperature of 445° C., the fluorine-free catalyst gives a lubricating oil yield of only 12% by weight.

#### Example 5

To demonstrate the importance of using alumina as a carrier, a Ni/W/F/SiO<sub>2</sub>-Al<sub>2</sub>O<sub>3</sub> catalyst containing 9% by weight of nickel, 17% by weight of tungsten and 2.5% by weight of fluorine on a carrier which comprised 26% by weight of alumina and the remainder being silica, was used for hydrocracking wax obtained during dewaxing of a residual lubricating oil fraction de-asphalted with propane (VI of the deasphalted oil after dewaxing at -19° C.:77). The residual lubricating oil fraction from which the wax (DAO slack wax) was prepared had been obtained during distillation under reduced pressure of an atmospheric distillation residue of a North African crude oil.

Dewaxing was carried out by cooling the oil to a temperature of -27° C. in the presence of a 1:1 mixture of methyl ethyl ketone and toluene.

Hydrocracking of the wax took place with the use of the catalyst in the sulfidic form at a temperature of 350° C., a pressure of 50 bar, a space velocity of 1 kg. 1<sup>-1</sup> hour<sup>-1</sup> and a hydrogen/feed ratio of 150 NL/kg. of oil.

From the hydrocracked product a residual fraction with an initial boiling point of 400° C. was separated by distillation and dewaxed by cooling the oil at a temperature of -27° C. in the presence of a 1:1 mixture of methyl ethyl ketone and toluene. The result was a dewaxed residual lubricating oil fraction in a yield of 20% by weight, based on feed, having a VI of 100, a kinematic viscosity at 98.0° C. of 16.9 cst. and a dynamic viscosity at -17.8° C. in excess of 200 P. These results demonstrate the unsuitability of a silica-alumina based catalyst for the present purpose since a 10W/30 oil cannot be prepared from the lubricating oil even by incorporating an additive package.

What is claimed is:

1. A process for preparing at least 15% wt. basis feed of a 10W/30 grade lubricating oil having a dynamic viscosity of at least 12 P and at most 24 P at -17.8° C. and a kinematic viscosity of at least 7.0 cst. at 98.9° C.

12

without the addition of a polymeric viscosity index improver which comprises: dewaxing a de-asphalted residual mineral oil fraction; obtaining a wax therefrom, more than 30% wt. of which boils above 520° C.; hydrocracking a feedstock consisting of said wax in the presence of a catalyst consisting of a catalytic amount of at least one metal sulfide selected from the group consisting of nickel and cobalt and of at least one metal sulfide selected from the group consisting of molybdenum and tungsten supported on a fluorine-containing alumina at a temperature between 325° C. and 425° C. and under conditions to form a liquid product containing 25-95% wt. of components having a boiling point over 400° C.; separating said liquid product by distillation into at least one light fraction and a residual fraction having an initial boiling point between 350° C. and 470° C.; dewaxing said residual reaction and recovering said 10W/30 grade lubricating oil.

2. The process of claim 1 wherein the aromatics have been removed from the de-asphalted residual oil fraction prior to dewaxing.

3. The process of claim 2 wherein the wax which is hydrocracked contains less than 35% wt. of oil.

4. The process of claim 2 wherein the wax which is hydrocracked has been obtained from a de-asphalted lubricating oil fraction which after dewaxing at -30° C. has a viscosity index of at least 55.

5. The process of claim 1 wherein the catalyst contains 0.025 to 0.8 gram atoms of nickel and/or cobalt and 0.05 to 0.5 gram atoms of molybdenum and/or tungsten per 100 grams of alumina.

6. The process of claim 4 wherein the atomic ratio between nickel and/or cobalt on the one hand and molybdenum and/or tungsten on the other is between 0.1:1 and 2:1.

7. The process of claim 1 wherein the catalyst contains 0.5 to 7% wt. of fluorine.

8. The process of claim 1 wherein the catalyst contains nickel and molybdenum or nickel and tungsten as catalytically active metal components.

9. The process of claim 1 wherein the hydrocracking process conditions include a pressure from 10 to 250 bar, a space velocity of 0.2 to 5 kg. of feed per litre of catalyst per hour and a hydrogen/feed ratio of 100 to 5000 NL of hydrogen per kg. of feed.

10. The process of claim 1 wherein the wax is converted by hydrocracking into a liquid product containing 40% to 70% wt. of components having a boiling point over 400° C. and the residual fraction separated by distillation has an initial boiling point between 390° C. and 450° C.

11. The process of claim 1 wherein a lubricating oil is prepared which meets the 10W/30 specification without additives having been incorporated therein.

#### References Cited

#### UNITED STATES PATENTS

|           |         |               |         |
|-----------|---------|---------------|---------|
| 2,817,693 | 12/1957 | Koome et al.  | 208-46  |
| 3,046,218 | 7/1962  | Henke et al.  | 208-109 |
| 3,520,796 | 7/1970  | Murphy et al. | 208-18  |

HERBERT LEVINE, Primary Examiner

U.S. Cl. X.R.

65 208-18